

## UNITED STATES PATENT OFFICE.

FRIEDRICH FISCHER AND HUGO GUNTRUM, OF ELBERFELD, GERMANY,  
ASSIGNORS TO FARBENFABRIKEN OF ELBERFELD CO., OF NEW YORK,  
N. Y., A CORPORATION OF NEW YORK.

## PROCESS OF DEVELOPING PHOTOGRAPHIC PICTURES.

SPECIFICATION forming part of Letters Patent No. 736,374, dated August 18, 1903.

Application filed February 20, 1903. Serial No. 144,332. (No specimens.)

To all whom it may concern:

Be it known that we, FRIEDRICH FISCHER and HUGO GUNTRUM, chemists, residing at Elberfeld, Germany, (assignors to the FAR-  
5 BENFABRIKEN OF ELBERFELD CO., of New York,) have invented certain new and useful Improvements in Processes of Developing Photographic Pictures, of which the following is a specification.

10 We have found that the m-amido-o-oxybenzyl sulfonic acid having the formula—



15 is especially suitable for developing photographic pictures. The production of the said amido-oxybenzyl sulfonic acid is described in a separate application for Letters Patent, filed February 20, 1903, Serial No. 144,332.

20 In carrying out the new process practically we can proceed as follows: Six grams of sodium sulfite are dissolved in one hundred cubic centimeters of water, and into the resulting solution one gram of m-amido-o-oxybenzyl sulfonic acid and six grams of potassium carbonate are introduced. The developer is thus ready for use.

25 In the above example sodium sulfite may

be replaced by potassium sulfite, sodium pyrosulfite, or potassium pyrosulfite or the like.

Having thus described our invention and 35 in what manner the same is to be performed, what we claim as new, and desire to secure by Letters Patent, is—

30 1. The herein-described process of developing photographic pictures, which consists 40 in subjecting them to the action of a solution containing amido-o-oxybenzyl sulfonic acid, substantially as hereinbefore described.

2. The process of developing photographic pictures which consists in subjecting them to 45 the action of a solution containing amido-o-oxybenzyl sulfonic acid, a preservative and an accelerator, substantially as hereinbefore described.

3. The process of developing photographic 50 pictures which consists in subjecting them to the action of a solution containing amido-o-oxybenzyl sulfonic acid, a sulfite and an alkali carbonate, substantially as hereinbefore described.

55 In testimony whereof we have signed our names in the presence of two subscribing witnesses.

FRIEDRICH FISCHER.  
HUGO GUNTRUM.

Witnesses:

OTTO KÖNIG,  
J. A. RITTERSHAUS.